



US009506297B2

(12) **United States Patent**  
**Overstreet**

(10) **Patent No.:** **US 9,506,297 B2**  
(45) **Date of Patent:** **\*Nov. 29, 2016**

(54) **ABRASIVE WEAR-RESISTANT MATERIALS AND EARTH-BORING TOOLS COMPRISING SUCH MATERIALS**

(71) Applicant: **Baker Hughes Incorporated**, Houston, TX (US)

(72) Inventor: **James L. Overstreet**, Tomball, TX (US)

(73) Assignee: **Baker Hughes Incorporated**, Houston, TX (US)

(\*) Notice: Subject to any disclaimer, the term of this patent is extended or adjusted under 35 U.S.C. 154(b) by 164 days.

This patent is subject to a terminal disclaimer.

(21) Appl. No.: **14/296,129**

(22) Filed: **Jun. 4, 2014**

(65) **Prior Publication Data**

US 2014/0284116 A1 Sep. 25, 2014

**Related U.S. Application Data**

(62) Division of application No. 12/350,761, filed on Jan. 8, 2009, now Pat. No. 8,758,462, which is a division of application No. 11/223,215, filed on Sep. 9, 2005, now Pat. No. 7,597,159.

(51) **Int. Cl.**

**C22C 29/08** (2006.01)  
**E21B 10/567** (2006.01)

(Continued)

(52) **U.S. Cl.**

CPC ..... **E21B 10/567** (2013.01); **B22F 7/062** (2013.01); **B24D 3/06** (2013.01); **C22C 29/08** (2013.01);

(Continued)

(58) **Field of Classification Search**

CPC ..... C22C 29/08  
See application file for complete search history.

(56) **References Cited**

U.S. PATENT DOCUMENTS

2,033,594 A 3/1936 Stoddy  
2,407,642 A 9/1946 Ashworth

(Continued)

FOREIGN PATENT DOCUMENTS

AU 695583 B2 8/1998  
CA 2212197 A1 2/1998

(Continued)

OTHER PUBLICATIONS

US 4,966,627, 10/1990, Keshavan et al. (withdrawn).

(Continued)

*Primary Examiner* — George Wyszomierski

*Assistant Examiner* — Ngoclan T Mai

(74) *Attorney, Agent, or Firm* — TraskBritt

(57) **ABSTRACT**

An abrasive wear-resistant material includes a matrix and sintered and cast tungsten carbide pellets. A device for use in drilling subterranean formations includes a first structure secured to a second structure with bonding material. An abrasive wear-resistant material covers the bonding material. The first structure may include a drill bit body and the second structure may include a cutting element. A method for applying an abrasive wear-resistant material to a drill bit includes providing a bit, mixing sintered and cast tungsten carbide pellets in a matrix material to provide a pre-application material, heating the pre-application material to melt the matrix material, applying the pre-application material to the bit, and solidifying the material. A method for securing a cutting element to a bit body includes providing an abrasive wear-resistant material to a surface of a drill bit that covers a brazing alloy disposed between the cutting element and the bit body.

**20 Claims, 8 Drawing Sheets**



|      |                    |                                                                                                                          |             |         |                 |  |
|------|--------------------|--------------------------------------------------------------------------------------------------------------------------|-------------|---------|-----------------|--|
| (51) | <b>Int. Cl.</b>    |                                                                                                                          |             |         |                 |  |
|      | <i>B22F 7/06</i>   | (2006.01)                                                                                                                | 4,667,756 A | 5/1987  | King et al.     |  |
|      | <i>C22C 32/00</i>  | (2006.01)                                                                                                                | 4,674,802 A | 6/1987  | McKenna et al.  |  |
|      | <i>E21B 10/46</i>  | (2006.01)                                                                                                                | 4,676,124 A | 6/1987  | Fischer         |  |
|      | <i>E21B 10/573</i> | (2006.01)                                                                                                                | 4,686,080 A | 8/1987  | Hara et al.     |  |
|      | <i>B24D 3/06</i>   | (2006.01)                                                                                                                | 4,694,919 A | 9/1987  | Barr            |  |
|      | <i>B22F 5/00</i>   | (2006.01)                                                                                                                | 4,726,432 A | 2/1988  | Scott et al.    |  |
| (52) | <b>U.S. Cl.</b>    |                                                                                                                          |             |         |                 |  |
|      | CPC .....          | <i>C22C 32/0052</i> (2013.01); <i>E21B 10/46</i> (2013.01); <i>E21B 10/573</i> (2013.01); <i>B22F 2005/001</i> (2013.01) | 4,743,515 A | 5/1988  | Fischer et al.  |  |
|      |                    |                                                                                                                          | 4,744,943 A | 5/1988  | Timm            |  |
|      |                    |                                                                                                                          | 4,762,028 A | 8/1988  | Regan           |  |
|      |                    |                                                                                                                          | 4,781,770 A | 11/1988 | Kar             |  |
|      |                    |                                                                                                                          | 4,809,903 A | 3/1989  | Eylon et al.    |  |
|      |                    |                                                                                                                          | 4,814,234 A | 3/1989  | Bird            |  |
|      |                    |                                                                                                                          | 4,836,307 A | 6/1989  | Keshavan et al. |  |
|      |                    |                                                                                                                          | 4,838,366 A | 6/1989  | Jones           |  |

(56) **References Cited**

## U.S. PATENT DOCUMENTS

|             |         |                      |             |         |                    |
|-------------|---------|----------------------|-------------|---------|--------------------|
| 2,660,405 A | 11/1953 | Scott et al.         | 4,923,511 A | 5/1990  | Krizan et al.      |
| 2,740,651 A | 4/1956  | Orloff               | 4,923,512 A | 5/1990  | Timm et al.        |
| 2,819,958 A | 1/1958  | Abkowitz et al.      | 4,933,240 A | 6/1990  | Barber, Jr.        |
| 2,819,959 A | 1/1958  | Abkowitz et al.      | 4,938,991 A | 7/1990  | Bird               |
| 2,906,654 A | 9/1959  | Abkowitz             | 4,944,774 A | 7/1990  | Keshavan et al.    |
| 2,961,312 A | 11/1960 | Elbaum               | 4,956,012 A | 9/1990  | Jacobs et al.      |
| 3,158,214 A | 11/1964 | Wisler et al.        | 4,968,348 A | 11/1990 | Abkowitz et al.    |
| 3,180,440 A | 4/1965  | Bridwell             | 5,000,273 A | 3/1991  | Horton et al.      |
| 3,260,579 A | 7/1966  | Scales et al.        | 5,010,225 A | 4/1991  | Carlin             |
| 3,368,881 A | 2/1968  | Abkowitz et al.      | 5,030,598 A | 7/1991  | Hsieh              |
| 3,471,921 A | 10/1969 | Feeenstra            | 5,032,352 A | 7/1991  | Meeks et al.       |
| 3,660,050 A | 5/1972  | Iler et al.          | 5,038,640 A | 8/1991  | Sullivan et al.    |
| 3,727,704 A | 4/1973  | Abplanalp            | 5,049,450 A | 9/1991  | Dorfman et al.     |
| 3,757,879 A | 9/1973  | Wilder et al.        | 5,051,112 A | 9/1991  | Keshavan et al.    |
| 3,768,984 A | 10/1973 | Foster, Jr.          | 5,089,182 A | 2/1992  | Findeisen et al.   |
| 3,790,353 A | 2/1974  | Jackson et al.       | 5,090,491 A | 2/1992  | Tibbitts et al.    |
| 3,800,891 A | 4/1974  | White et al.         | 5,101,692 A | 4/1992  | Simpson            |
| 3,868,235 A | 2/1975  | Held                 | 5,150,636 A | 9/1992  | Hill               |
| 3,942,954 A | 3/1976  | Frehn                | 5,152,194 A | 10/1992 | Keshavan et al.    |
| 3,987,859 A | 10/1976 | Lichte               | 5,161,898 A | 11/1992 | Drake              |
| 3,989,554 A | 11/1976 | Wisler               | 5,186,267 A | 2/1993  | White              |
| 4,013,453 A | 3/1977  | Patel                | 5,232,522 A | 8/1993  | Doktycz et al.     |
| 4,017,480 A | 4/1977  | Baum                 | 5,242,017 A | 9/1993  | Hailey             |
| 4,043,611 A | 8/1977  | Wallace              | 5,250,355 A | 10/1993 | Newman et al.      |
| 4,047,828 A | 9/1977  | Makely               | 5,281,260 A | 1/1994  | Kumar et al.       |
| 4,059,217 A | 11/1977 | Woodward             | 5,286,685 A | 2/1994  | Schoennahl et al.  |
| 4,094,709 A | 6/1978  | Rozmus               | 5,291,807 A | 3/1994  | Vanderford et al.  |
| 4,128,136 A | 12/1978 | Generoux             | 5,311,958 A | 5/1994  | Isbell et al.      |
| 4,173,457 A | 11/1979 | Smith                | 5,328,763 A | 7/1994  | Terry              |
| 4,198,233 A | 4/1980  | Frehn                | 5,348,806 A | 9/1994  | Kojo et al.        |
| 4,221,270 A | 9/1980  | Vezirian             | 5,373,907 A | 12/1994 | Weaver             |
| 4,229,638 A | 10/1980 | Lichte               | 5,375,759 A | 12/1994 | Hiraishi et al.    |
| 4,233,720 A | 11/1980 | Rozmus               | 5,425,288 A | 6/1995  | Evans              |
| 4,243,727 A | 1/1981  | Wisler et al.        | 5,433,280 A | 7/1995  | Smith              |
| 4,252,202 A | 2/1981  | Purser, Sr.          | 5,439,068 A | 8/1995  | Huffstutler et al. |
| 4,255,165 A | 3/1981  | Dennis et al.        | 5,443,337 A | 8/1995  | Katayama           |
| 4,262,761 A | 4/1981  | Crow                 | 5,479,997 A | 1/1996  | Scott et al.       |
| 4,306,139 A | 12/1981 | Shinozaki et al.     | 5,482,670 A | 1/1996  | Hong               |
| 4,341,557 A | 7/1982  | Lizenby              | 5,484,468 A | 1/1996  | Ostlund et al.     |
| 4,389,952 A | 6/1983  | Dreier et al.        | 5,492,186 A | 2/1996  | Overstreet et al.  |
| 4,398,952 A | 8/1983  | Drake                | 5,506,055 A | 4/1996  | Dorfman et al.     |
| 4,414,029 A | 11/1983 | Newman et al.        | 5,535,838 A | 7/1996  | Keshavan et al.    |
| 4,455,278 A | 6/1984  | van Nederveen et al. | 5,543,235 A | 8/1996  | Mirchandani et al. |
| 4,499,048 A | 2/1985  | Hanejko              | 5,544,550 A | 8/1996  | Smith              |
| 4,499,795 A | 2/1985  | Radtke               | 5,560,440 A | 10/1996 | Tibbitts           |
| 4,499,958 A | 2/1985  | Radtke et al.        | 5,586,612 A | 12/1996 | Isbell et al.      |
| 4,526,748 A | 7/1985  | Rozmus               | 5,589,268 A | 12/1996 | Kelley et al.      |
| 4,547,337 A | 10/1985 | Rozmus               | 5,593,474 A | 1/1997  | Keshavan et al.    |
| 4,552,232 A | 11/1985 | Frear                | 5,611,251 A | 3/1997  | Katayama           |
| 4,554,130 A | 11/1985 | Ecer                 | 5,612,264 A | 3/1997  | Nilsson et al.     |
| 4,562,892 A | 1/1986  | Ecer                 | 5,641,251 A | 6/1997  | Leins et al.       |
| 4,562,990 A | 1/1986  | Rose                 | 5,641,921 A | 6/1997  | Dennis et al.      |
| 4,579,713 A | 4/1986  | Lueth                | 5,653,299 A | 8/1997  | Sreshta et al.     |
| 4,596,694 A | 6/1986  | Rozmus               | 5,662,183 A | 9/1997  | Fang               |
| 4,597,456 A | 7/1986  | Ecer                 | 5,663,512 A | 9/1997  | Schader et al.     |
| 4,597,730 A | 7/1986  | Rozmus               | 5,666,864 A | 9/1997  | Tibbitts           |
| 4,611,673 A | 9/1986  | Childers et al.      | 5,667,903 A | 9/1997  | Boyce              |
| 4,630,692 A | 12/1986 | Ecer                 | 5,677,042 A | 10/1997 | Massa et al.       |
| 4,630,693 A | 12/1986 | Goodfellow           | 5,679,445 A | 10/1997 | Massa et al.       |
| 4,656,002 A | 4/1987  | Lizenby et al.       | 5,697,046 A | 12/1997 | Conley             |
| 4,666,797 A | 5/1987  | Newman et al.        | 5,697,462 A | 12/1997 | Grimes et al.      |

| (56)                  | References Cited            |                 |                            |  |
|-----------------------|-----------------------------|-----------------|----------------------------|--|
| U.S. PATENT DOCUMENTS |                             |                 |                            |  |
| 5,732,783 A           | 3/1998 Truax et al.         | 6,576,182 B1    | 6/2003 Ravagni et al.      |  |
| 5,733,649 A           | 3/1998 Kelley et al.        | 6,589,640 B2    | 7/2003 Griffin et al.      |  |
| 5,733,664 A           | 3/1998 Kelley et al.        | 6,599,467 B1    | 7/2003 Yamaguchi et al.    |  |
| 5,740,872 A           | 4/1998 Smith                | 6,607,693 B1    | 8/2003 Saito et al.        |  |
| 5,753,160 A           | 5/1998 Takeuchi et al.      | 6,615,936 B1    | 9/2003 Mourik et al.       |  |
| 5,755,298 A           | 5/1998 Langford, Jr. et al. | 6,651,756 B1    | 11/2003 Costo, Jr. et al.  |  |
| 5,765,095 A           | 6/1998 Flak et al.          | 6,655,481 B2    | 12/2003 Findley            |  |
| 5,776,593 A           | 7/1998 Massa et al.         | 6,659,206 B2    | 12/2003 Liang et al.       |  |
| 5,778,301 A           | 7/1998 Hong                 | 6,663,688 B2    | 12/2003 Findeisen et al.   |  |
| 5,789,686 A           | 8/1998 Massa et al.         | 6,685,880 B2    | 2/2004 Engström et al.     |  |
| 5,791,422 A           | 8/1998 Liang et al.         | 6,725,952 B2    | 4/2004 Singh               |  |
| 5,791,423 A           | 8/1998 Overstreet et al.    | 6,742,608 B2    | 6/2004 Murdoch             |  |
| 5,792,403 A           | 8/1998 Massa et al.         | 6,742,611 B1    | 6/2004 Illerhaus et al.    |  |
| 5,806,934 A           | 9/1998 Massa et al.         | 6,756,009 B2    | 6/2004 Sim et al.          |  |
| 5,830,256 A           | 11/1998 Northrop et al.     | 6,766,870 B2    | 7/2004 Overstreet          |  |
| 5,856,626 A           | 1/1999 Fischer et al.       | 6,772,849 B2    | 8/2004 Oldham et al.       |  |
| 5,865,571 A           | 2/1999 Tankala et al.       | 6,782,958 B2    | 8/2004 Liang et al.        |  |
| 5,880,382 A           | 3/1999 Fang et al.          | 6,849,231 B2    | 2/2005 Kojima              |  |
| 5,893,204 A           | 4/1999 Symonds              | 6,861,612 B2    | 3/2005 Bolton et al.       |  |
| 5,896,940 A           | 4/1999 Pietrobelli et al.   | 6,918,942 B2    | 7/2005 Hatta et al.        |  |
| 5,897,830 A           | 4/1999 Abkowitz et al.      | 6,948,403 B2    | 9/2005 Singh               |  |
| 5,904,212 A           | 5/1999 Arfele               | 6,984,454 B2    | 1/2006 Majagi              |  |
| 5,921,330 A           | 7/1999 Sue et al.           | 7,044,243 B2    | 5/2006 Kembaiyan et al.    |  |
| 5,924,502 A           | 7/1999 Arfele et al.        | 7,048,081 B2    | 5/2006 Smith et al.        |  |
| 5,954,147 A           | 9/1999 Overstreet           | 7,240,746 B2    | 7/2007 Overstreet et al.   |  |
| 5,957,006 A           | 9/1999 Smith                | 7,537,159 B2    | 5/2009 Mugica et al.       |  |
| 5,963,775 A           | 10/1999 Fang                | 7,597,159 B2    | 10/2009 Overstreet         |  |
| 5,967,248 A           | 10/1999 Drake et al.        | 7,644,786 B2    | 1/2010 Lockstedt et al.    |  |
| 5,988,302 A           | 11/1999 Sreshta et al.      | 7,703,555 B2    | 4/2010 Overstreet          |  |
| 5,988,303 A           | 11/1999 Arfele              | 7,776,256 B2    | 8/2010 Smith               |  |
| 6,009,961 A           | 1/2000 Pietrobelli et al.   | 7,997,359 B2    | 8/2011 Eason et al.        |  |
| 6,029,544 A           | 2/2000 Katayama             | 8,388,723 B2    | 3/2013 Overstreet          |  |
| 6,045,750 A           | 4/2000 Drake et al.         | 2001/0015290 A1 | 8/2001 Sue et al.          |  |
| 6,051,171 A           | 4/2000 Takeuchi et al.      | 2001/0017224 A1 | 8/2001 Evans et al.        |  |
| 6,063,333 A           | 5/2000 Dennis               | 2002/0004105 A1 | 1/2002 Kunze et al.        |  |
| 6,068,070 A           | 5/2000 Scott                | 2003/0000339 A1 | 1/2003 Findeisen et al.    |  |
| 6,073,518 A           | 6/2000 Chow et al.          | 2003/0010409 A1 | 1/2003 Kunze et al.        |  |
| 6,086,980 A           | 7/2000 Foster et al.        | 2003/0079565 A1 | 5/2003 Liang et al.        |  |
| 6,089,123 A           | 7/2000 Chow et al.          | 2003/0079916 A1 | 5/2003 Oldham et al.       |  |
| 6,099,664 A           | 8/2000 Davies et al.        | 2004/0013558 A1 | 1/2004 Kondoh et al.       |  |
| 6,124,564 A           | 9/2000 Sue et al.           | 2004/0060742 A1 | 4/2004 Kembaiyan et al.    |  |
| 6,131,677 A           | 10/2000 Arfele et al.       | 2004/0196638 A1 | 10/2004 Lee et al.         |  |
| 6,148,936 A           | 11/2000 Evans et al.        | 2004/0234821 A1 | 11/2004 Majagi             |  |
| 6,196,338 B1          | 3/2001 Slaughter et al.     | 2004/0243241 A1 | 12/2004 Istephanous et al. |  |
| 6,200,514 B1          | 3/2001 Meister              | 2004/0245022 A1 | 12/2004 Izaguirre et al.   |  |
| 6,206,115 B1          | 3/2001 Overstreet et al.    | 2004/0245024 A1 | 12/2004 Kembaiyan          |  |
| RE37,127 E            | 4/2001 Schader et al.       | 2005/0000317 A1 | 1/2005 Liang et al.        |  |
| 6,209,420 B1          | 4/2001 Butcher et al.       | 2005/0008524 A1 | 1/2005 Testani             |  |
| 6,214,134 B1          | 4/2001 Eylon et al.         | 2005/0072496 A1 | 4/2005 Hwang et al.        |  |
| 6,214,287 B1          | 4/2001 Waldenström          | 2005/0084407 A1 | 4/2005 Myrick              |  |
| 6,220,117 B1          | 4/2001 Butcher              | 2005/0117984 A1 | 6/2005 Eason et al.        |  |
| 6,227,188 B1          | 5/2001 Tankala et al.       | 2005/0126334 A1 | 6/2005 Mirchandani         |  |
| 6,228,139 B1          | 5/2001 Oskarsson            | 2005/0211475 A1 | 9/2005 Mirchandani et al.  |  |
| 6,234,261 B1          | 5/2001 Evans et al.         | 2005/0247491 A1 | 11/2005 Mirchandani et al. |  |
| 6,241,036 B1          | 6/2001 Lovato et al.        | 2005/0268746 A1 | 12/2005 Abkowitz et al.    |  |
| 6,248,149 B1          | 6/2001 Massey et al.        | 2006/0016521 A1 | 1/2006 Hanusiak et al.     |  |
| 6,254,658 B1          | 7/2001 Taniuchi et al.      | 2006/0032677 A1 | 2/2006 Azar et al.         |  |
| 6,287,360 B1          | 9/2001 Kembaiyan et al.     | 2006/0043648 A1 | 3/2006 Takeuchi et al.     |  |
| 6,290,438 B1          | 9/2001 Papajewski           | 2006/0057017 A1 | 3/2006 Woodfield et al.    |  |
| 6,293,986 B1          | 9/2001 Rödiger et al.       | 2006/0131081 A1 | 6/2006 Mirchandani et al.  |  |
| 6,348,110 B1          | 2/2002 Evans                | 2006/0185908 A1 | 8/2006 Kembaiyan et al.    |  |
| 6,349,780 B1          | 2/2002 Beuershausen         | 2007/0042217 A1 | 2/2007 Fang et al.         |  |
| 6,360,832 B1          | 3/2002 Overstreet et al.    | 2007/0056776 A1 | 3/2007 Overstreet et al.   |  |
| 6,375,706 B2          | 4/2002 Kembaiyan et al.     | 2007/0056777 A1 | 3/2007 Overstreet          |  |
| 6,450,271 B1          | 9/2002 Tibbitts             | 2007/0102198 A1 | 5/2007 Oxford et al.       |  |
| 6,453,899 B1          | 9/2002 Tselesin             | 2007/0102199 A1 | 5/2007 Smith et al.        |  |
| 6,454,025 B1          | 9/2002 Runquist et al.      | 2007/0102200 A1 | 5/2007 Choe et al.         |  |
| 6,454,028 B1          | 9/2002 Evans                | 2007/0163812 A1 | 7/2007 Overstreet et al.   |  |
| 6,454,030 B1          | 9/2002 Findley et al.       | 2007/0205023 A1 | 9/2007 Hoffmaster et al.   |  |
| 6,458,471 B2          | 10/2002 Lovato et al.       | 2008/0053709 A1 | 3/2008 Lockstedt et al.    |  |
| 6,474,425 B1          | 11/2002 Truax et al.        | 2008/0073125 A1 | 3/2008 Eason et al.        |  |
| 6,500,226 B1          | 12/2002 Dennis              | 2008/0083568 A1 | 4/2008 Overstreet          |  |
| 6,511,265 B1          | 1/2003 Mirchandani et al.   | 2008/0164070 A1 | 7/2008 Keshavan et al.     |  |
| 6,568,491 B1          | 5/2003 Matthews, III et al. | 2009/0113811 A1 | 5/2009 Overstreet          |  |
| 6,575,350 B2          | 6/2003 Evans et al.         |                 |                            |  |

(56)

**References Cited****U.S. PATENT DOCUMENTS**

2010/0000798 A1 1/2010 Patel  
 2010/0132265 A1 6/2010 Overstreet

**FOREIGN PATENT DOCUMENTS**

|    |               |         |
|----|---------------|---------|
| CN | 1562550 A     | 1/2005  |
| EP | 264674        | 4/1988  |
| EP | 453428        | 10/1991 |
| EP | 995876        | 4/2000  |
| EP | 1244531 A1    | 10/2004 |
| GB | 945227 A      | 12/1963 |
| GB | 1070039 A     | 5/1967  |
| GB | 2104101 A     | 3/1983  |
| GB | 2203774 A     | 10/1988 |
| GB | 2295157 A     | 5/1996  |
| GB | 2352727 A     | 2/2001  |
| GB | 2357788 A     | 7/2001  |
| GB | 2385350 A     | 8/2003  |
| GB | 2393449 A     | 3/2004  |
| JP | 10219385 A    | 8/1998  |
| WO | 03049889 A2   | 6/2003  |
| WO | 2004053197 A2 | 6/2004  |
| WO | 2006099629 A1 | 9/2006  |
| WO | 2007030707 A1 | 3/2007  |

**OTHER PUBLICATIONS**

Boron Carbide Nozzles and Inserts, Seven Stars International webpage <http://www.concentric.net/~ctkang/nozzle.shtml>, printed Sep. 7, 2006.

“Heat Treating of Titanium and Titanium Alloys,” Key to Metals website article, [www.key-to-metals.com](http://www.key-to-metals.com), visited Sep. 21, 2006.

Alman, D.E., et al., “The Abrasive Wear of Sintered Titanium Matrix-Ceramic Particle Reinforced Composites,” *Wear*, 225-229 (1999), pp. 629-639.

B & W Metals, “Today we’re more then just Kutrite © composite rods . . . much more!,” Houston, Texas, 2 pages, visited Jun. 12, 2008.

B & W Metals, Kutrite, <http://www.bwmetals.com>, 1 page, visited Jun. 12, 2008.

Canadian Office Action for Canadian Application No. 2,621,421 dated Sep. 14, 2011, 3 pages.

Choe, Heeman, et al., “Effect of Tungsten Additions on the Mechanical Properties of Ti-6Al1-4V,” *Material Science and Engineering*, A 396 (2005), pp. 99-106, Elsevier.

Diamond Innovations, “Composite Diamond Coatings, Superhard Protection of Wear Parts New Coating and Service Parts from Diamond Innovations” brochure, 2004.

Gale, W.F., et al., *Smithells Metals Reference Book*, Eighth Edition, 2003, p. 2,117, Elsevier Butterworth Heinemann.

Miserez, A., et al. “Particle Reinforced Metals of High Ceramic Content,” *Material Science and Engineering A* 387-389 (2004), pp. 822-831, Elsevier.

PCT International Search Report for WO 2007/030707 A1 (PCT/US2006/035010), mailed Dec. 27, 2006 (3 pages).

PCT International Search Report for WO 2008/027484 A1 (PCT/US2007/019085), mailed Jan. 31, 2008 (4 pages).

PCT International Application Search Report for International Application No. PCT/US2009/048232 mailed Feb. 2, 2010, 5 pages.

PCT International Search Report for PCT/US2007/021072, mailed Feb. 27, 2008.

PCT International Search Report for counterpart PCT International Application No. PCT/US2007/023275, mailed Apr. 11, 2008.

PCT International Search Report for PCT Counterpart Application No. PCT/US2006/043670, mailed Apr. 2, 2007.

PCT International Search Report for PCT/US2007/021071, mailed Feb. 6, 2008.

PCT International Search Report PCT Counterpart Application No. PCT/US2006/043669, mailed Apr. 13, 2007.

PCT Written Opinion for counterpart PCT International Application No. PCT/US2007/023275, mailed Apr. 11, 2008.

PCT Written Opinion for International Application No. PCT/US2006/035010, mailed Dec. 27, 2006.

PCT Written Opinion for International Application No. PCT/US2007/019085, mailed Jan. 31, 2008.

PCT Written Opinion for PCT Counterpart Application No. PCT/US2006/043670, mailed Apr. 2, 2007.

PCT Written Opinion for PCT/US2007/021071, mailed Feb. 6, 2008.

PCT Written Opinion for PCT/US2007/021072, mailed Feb. 27, 2008.

PCT Written Opinion Report PCT Counterpart Application No. PCT/US2006/043669, mailed Apr. 13, 2007.

PCT Written Opinion for International Application No. PCT/US2009/048232 mailed Feb. 2, 2010, 4 pages.

Reed, James S., “Chapter 13: Particle Packing Characteristics,” *Principles of Ceramics Processing*, Second Edition, John Wiley & Sons, Inc. (1995), pp. 215-227.

Smith International, Inc., Smith Bits Product Catalog 2005-2006, p. 45.

Wall Colmonoy “Colmonoy Alloy Selector Chart” 2003, pp. 1 and 2.

Warrier, S.G., et al., “Infiltration of Titanium Alloy-Matrix Composites,” *Journal of Materials Science Letters*, 12 (1993), pp. 865-868, Chapman & Hall.

[www.matweb.com](http://www.matweb.com) “Wall Comonoy Colmonoy 4 Hard-surfacing alloy with chromium boride” from [www.matweb.com](http://www.matweb.com), 1 page, printed Mar. 19, 2009.

Zhou et al., Laser Melted Alloys and WC Composite Coating and its Applications, *Sichuan Binggong Xuebao* (1998), 19(2), 20-22.



**FIG. 1**  
**(PRIOR ART)**



**FIG. 2**  
**(PRIOR ART)**



**FIG. 3**  
(PRIOR ART)



**FIG. 4**  
(PRIOR ART)

**FIG. 5****FIG. 6**

**FIG. 7A**



**FIG. 7B**



**FIG. 7C**

**FIG. 8A****FIG. 8B**



*FIG. 9*

## 1

**ABRASIVE WEAR-RESISTANT MATERIALS  
AND EARTH-BORING TOOLS COMPRISING  
SUCH MATERIALS**

**CROSS-REFERENCE TO RELATED  
APPLICATIONS**

This application is a divisional of U.S. patent application Ser. No. 12/350,761, filed Jan. 8, 2009, now U.S. Pat. No. 8,758,462, issued Jun. 24, 2014, which is a divisional of U.S. patent application Ser. No. 11/223,215, filed Sep. 9, 2005, now U.S. Pat. No. 7,597,159, issued Oct. 6, 2009, the disclosure of each of which is incorporated in its entirety by reference herein.

**FIELD**

The present invention generally relates to earth-boring drill bits and other tools that may be used to drill subterranean formations, and to abrasive, wear-resistant hardfacing materials that may be used on surfaces of such earth-boring drill bits. The present invention also relates to methods for applying abrasive wear-resistant hardfacing materials to surfaces of earth-boring drill bits, and to methods for securing cutting elements to an earth-boring drill bit.

**BACKGROUND**

A typical fixed-cutter, or “drag,” rotary drill bit for drilling subterranean formations includes a bit body having a face region thereon carrying cutting elements for cutting into an earth formation. The bit body may be secured to a hardened steel shank having a threaded pin connection for attaching the drill bit to a drill string that includes tubular pipe segments coupled end to end between the drill bit and other drilling equipment. Equipment such as a rotary table or top drive may be used for rotating the tubular pipe and drill bit. Alternatively, the shank may be coupled directly to the drive shaft of a down-hole motor to rotate the drill bit.

Typically, the bit body of a drill bit is formed from steel or a combination of a steel blank embedded in a matrix material that includes hard particulate material, such as tungsten carbide, infiltrated with a binder material such as a copper alloy. A steel shank may be secured to the bit body after the bit body has been formed. Structural features may be provided at selected locations on and in the bit body to facilitate the drilling process. Such structural features may include, for example, radially and longitudinally extending blades, cutting element pockets, ridges, lands, nozzle displacements, and drilling fluid courses and passages. The cutting elements generally are secured within pockets that are machined into blades located on the face region of the bit body.

Generally, the cutting elements of a fixed-cutter type drill bit each include a cutting surface comprising a hard, super-abrasive material such as mutually bound particles of polycrystalline diamond. Such “polycrystalline diamond compact” (PDC) cutters have been employed on fixed-cutter rotary drill bits in the oil and gas well drilling industries for several decades.

FIG. 1 illustrates a conventional fixed-cutter rotary drill bit 10 generally according to the description above. The rotary drill bit 10 includes a bit body 12 that is coupled to a steel shank 14. A bore (not shown) is formed longitudinally through a portion of the drill bit 10 for communicating drilling fluid to a face 20 of the drill bit 10 via nozzles 19 during drilling operations. Cutting elements 22 (typically

## 2

polycrystalline diamond compact (PDC) cutting elements) generally are bonded to the bit face 20 of the bit body 12 by methods such as brazing, adhesive bonding, or mechanical affixation.

5 A drill bit 10 may be used numerous times to perform successive drilling operations during which the surfaces of the bit body 12 and cutting elements 22 may be subjected to extreme forces and stresses as the cutting elements 22 of the drill bit 10 shear away the underlying earth formation. These 10 extreme forces and stresses cause the cutting elements 22 and the surfaces of the bit body 12 to wear. Eventually, the cutting elements 22 and the surfaces of the bit body 12 may wear to an extent at which the drill bit 10 is no longer suitable for use.

15 FIG. 2 is an enlarged view of a PDC cutting element 22 like those shown in FIG. 1 secured to the bit body 12. Cutting elements 22 generally are not integrally formed with the bit body 12. Typically, the cutting elements 22 are fabricated separately from the bit body 12 and secured 20 within pockets 21 formed in the outer surface of the bit body 12. A bonding material 24 such as an adhesive or, more typically, a braze alloy may be used to secure the cutting elements 22 to the bit body 12 as previously discussed herein. Furthermore, if the cutting element 22 is a PDC 25 cutter, the cutting element 22 may include a polycrystalline diamond compact table 28 secured to a cutting element body or substrate 23, which may be unitary or comprise two components bound together.

The bonding material 24 typically is much less resistant to 30 wear than are other portions and surfaces of the drill bit 10 and of cutting elements 22. During use, small vugs, voids and other defects may be formed in exposed surfaces of the bonding material 24 due to wear. Solids-laden drilling fluids and formation debris generated during the drilling process 35 may further erode, abrade and enlarge the small vugs and voids in the bonding material 24. The entire cutting element 22 may separate from the drill bit body 12 during a drilling operation if enough bonding material 24 is removed. Loss of a cutting element 22 during a drilling operation can lead to 40 rapid wear of other cutting elements and catastrophic failure of the entire drill bit 10. Therefore, there is a need in the art for an effective method for preventing the loss of cutting elements during drilling operations.

The materials of an ideal drill bit must be extremely hard 45 to efficiently shear away the underlying earth formations without excessive wear. Due to the extreme forces and stresses to which drill bits are subjected during drilling operations, the materials of an ideal drill bit must simultaneously exhibit high fracture toughness. In practicality, 50 however, materials that exhibit extremely high hardness tend to be relatively brittle and do not exhibit high fracture toughness, while materials exhibiting high fracture toughness tend to be relatively soft and do not exhibit high hardness. As a result, a compromise must be made between 55 hardness and fracture toughness when selecting materials for use in drill bits.

In an effort to simultaneously improve both the hardness and fracture toughness of earth-boring drill bits, composite materials have been applied to the surfaces of drill bits that 60 are subjected to extreme wear. These composite materials are often referred to as “hard-facing” materials and typically include at least one phase that exhibits relatively high hardness and another phase that exhibits relatively high fracture toughness.

65 FIG. 3 is a representation of a photomicrograph of a polished and etched surface of a conventional hard-facing material. The hard-facing material includes tungsten carbide

particles **40** substantially randomly dispersed throughout an iron-based matrix of matrix material **46**. The tungsten carbide particles **40** exhibit relatively high hardness, while the matrix material **46** exhibits relatively high fracture toughness.

Tungsten carbide particles **40** used in hard-facing materials may comprise one or more of cast tungsten carbide particles, sintered tungsten carbide particles, and macrocrystalline tungsten carbide particles. The tungsten carbide system includes two stoichiometric compounds, WC and W<sub>2</sub>C, with a continuous range of compositions therebetween. Cast tungsten carbide generally includes a eutectic mixture of the WC and W<sub>2</sub>C compounds. Sintered tungsten carbide particles include relatively smaller particles of WC bonded together by a matrix material. Cobalt and cobalt alloys are often used as matrix materials in sintered tungsten carbide particles. Sintered tungsten carbide particles can be formed by mixing together a first powder that includes the relatively smaller tungsten carbide particles and a second powder that includes cobalt particles. The powder mixture is formed in a "green" state. The green powder mixture then is sintered at a temperature near the melting temperature of the cobalt particles to form a matrix of cobalt material surrounding the tungsten carbide particles to form particles of sintered tungsten carbide. Finally, macrocrystalline tungsten carbide particles generally consist of single crystals of WC.

Various techniques known in the art may be used to apply a hard-facing material such as that represented in FIG. 3 to a surface of a drill bit. The rod may be configured as a hollow, cylindrical tube formed from the matrix material of the hard-facing material that is filled with tungsten carbide particles. At least one end of the hollow, cylindrical tube may be sealed. The sealed end of the tube then may be melted or welded onto the desired surface on the drill bit. As the tube melts, the tungsten carbide particles within the hollow, cylindrical tube mix with the molten matrix material as it is deposited onto the drill bit. An alternative technique involves forming a cast rod of the hard-facing material and using either an arc or a torch to apply or weld hard-facing material disposed at an end of the rod to the desired surface on the drill bit.

Arc welding techniques also may be used to apply a hard-facing material to a surface of a drill bit. For example, a plasma-transferred arc may be established between an electrode and a region on a surface of a drill bit on which it is desired to apply a hard-facing material. A powder mixture including both particles of tungsten carbide and particles of matrix material then may be directed through or proximate the plasma transferred arc onto the region of the surface of the drill bit. The heat generated by the arc melts at least the particles of matrix material to form a weld pool on the surface of the drill bit, which subsequently solidifies to form the hard-facing material layer on the surface of the drill bit.

When a hard-facing material is applied to a surface of a drill bit, relatively high temperatures are used to melt at least the matrix material. At these relatively high temperatures, atomic diffusion may occur between the tungsten carbide particles and the matrix material. In other words, after applying the hard-facing material, at least some atoms originally contained in a tungsten carbide particle (tungsten and carbon for example) may be found in the matrix material surrounding the tungsten carbide particle. In addition, at least some atoms originally contained in the matrix material (iron for example) may be found in the tungsten carbide particles. FIG. 4 is an enlarged view of a tungsten carbide particle **40** shown in FIG. 3. At least some atoms originally contained in the tungsten carbide particle **40** (tungsten and

carbon for example) may be found in a region **47** of the matrix material **46** immediately surrounding the tungsten carbide particle **40**. The region **47** roughly includes the region of the matrix material **46** enclosed within the phantom line **48**. In addition, at least some atoms originally contained in the matrix material **46** (iron for example) may be found in a peripheral or outer region **41** of the tungsten carbide particle **40**. The outer region **41** roughly includes the region of the tungsten carbide particle **40** outside the phantom line **42**.

Atomic diffusion between the tungsten carbide particle **40** and the matrix material **46** may embrittle the matrix material **46** in the region **47** surrounding the tungsten carbide particle **40** and reduce the hardness of the tungsten carbide particle **40** in the outer region **41** thereof, reducing the overall effectiveness of the hard-facing material. Therefore, there is a need in the art for abrasive wear-resistant hardfacing materials that include a matrix material that allows for atomic diffusion between tungsten carbide particles and the matrix material to be minimized. There is also a need in the art for methods of applying such abrasive wear-resistant hardfacing materials, and for drill bits and drilling tools that include such materials.

#### BRIEF SUMMARY

In one aspect, the present invention includes an abrasive wear-resistant material that includes a matrix material, a plurality of -20 ASTM (American Society for Testing and Materials) mesh sintered tungsten carbide pellets, and a plurality of -100 ASTM mesh sintered tungsten carbide pellets. The tungsten carbide pellets are substantially randomly dispersed throughout the matrix material. The matrix material includes at least 75% nickel by weight and has a melting point of less than about 1100° C. Each sintered tungsten pellet includes a plurality of tungsten carbide particles bonded together with a binder alloy having a melting point greater than about 1200° C. In pre-application ratios, the matrix material comprises between about 30% and about 50% by weight of the abrasive wear resistant material, the plurality of sintered tungsten carbide pellets comprises between about 30% and about 55% by weight of the abrasive wear resistant material, and the plurality of cast tungsten carbide pellets comprises between about 15% and about 35% by weight of the abrasive wear resistant material.

In another aspect, the present invention includes a device for use in drilling subterranean formations. The device includes a first structure, a second structure secured to the structure along an interface, and a bonding material disposed between the first structure and the second structure at the interface. The bonding material secures the first and second structures together. The device further includes an abrasive wear-resistant material disposed on a surface of the device. At least a continuous portion of the wear-resistant material is bonded to a surface of the first structure and a surface of the second structure. The continuous portion of the wear-resistant material extends at least over the interface between the first structure and the second structure and covers the bonding material. The abrasive wear-resistant material includes a matrix material having a melting temperature of less than about 1100° C., a plurality of sintered tungsten carbide pellets substantially randomly dispersed throughout the matrix material, and a plurality of cast tungsten carbide pellets substantially randomly dispersed throughout the matrix material.

In an additional aspect, the present invention includes a rotary drill bit for drilling subterranean formations that

includes a bit body and at least one cutting element secured to the bit body along an interface. As used herein, the term "drill bit" includes and encompasses drilling tools of any configuration, including core bits, eccentric bits, bicenter bits, reamers, mills, drag bits, roller cone bits, and other such structures known in the art. A brazing alloy is disposed between the bit body and the at least one cutting element at the interface and secures the at least one cutting element to the bit body. An abrasive wear-resistant material includes, in pre-application ratios, a matrix material that comprises between about 30% and about 50% by weight of the abrasive wear-resistant material, a plurality of -20 ASTM mesh sintered tungsten carbide pellets that comprises between about 30% and about 55% by weight of the abrasive wear-resistant material, and a plurality of -100 ASTM mesh cast tungsten carbide pellets that comprises between about 15% and about 35% by weight of the abrasive wear-resistant material. The tungsten carbide pellets are substantially randomly dispersed throughout the matrix material. The matrix material includes at least 75% nickel by weight and has a melting point of less than about 1100° C. Each sintered tungsten pellet includes a plurality of tungsten carbide particles bonded together with a binder alloy having a melting point greater than about 1200° C.

In yet another aspect, the present invention includes a method for applying an abrasive wear-resistant material to a surface of a drill bit for drilling subterranean formations. The method includes providing a drill bit including a bit body having an outer surface, mixing a plurality of -20 ASTM mesh sintered tungsten carbide pellets and a plurality of -100 ASTM mesh cast tungsten carbide pellets in a matrix material to provide a pre-application abrasive wear resistant material, and melting the matrix material. The molten matrix material, at least some of the sintered tungsten carbide pellets, and at least some of the cast tungsten carbide pellets are applied to at least a portion of the outer surface of the drill bit, and the molten matrix material is solidified. The matrix material includes at least 75% nickel by weight and has a melting point of less than about 1100° C. Each sintered tungsten pellet includes a plurality of tungsten carbide particles bonded together with a binder alloy having a melting point greater than about 1200° C. The matrix material comprises between about 30% and about 50% by weight of the pre-application abrasive wear-resistant material, the plurality of sintered tungsten carbide pellets comprises between about 30% and about 55% by weight of the pre-application abrasive wear-resistant material, and the plurality of cast tungsten carbide pellets comprises between about 15% and about 35% by weight of the pre-application abrasive wear-resistant material.

In another aspect, the present invention includes a method for securing a cutting element to a bit body of a rotary drill bit. The method includes providing a rotary drill bit including a bit body having an outer surface including a pocket therein that is configured to receive a cutting element, and positioning a cutting element within the pocket. A brazing alloy is provided, melted, and applied to adjacent surfaces of the cutting element and the outer surface of the bit body within the pocket defining an interface therebetween and solidified. An abrasive wear-resistant material is applied to a surface of the drill bit. At least a continuous portion of the abrasive wear-resistant material is bonded to a surface of the cutting element and a portion of the outer surface of the bit body. The continuous portion extends over at least the interface between the cutting element and the outer surface of the bit body and covers the brazing alloy. In pre-application ratios, the abrasive wear resistant material comprises

a matrix material, a plurality of sintered tungsten carbide pellets, and a plurality of cast tungsten carbide pellets. The matrix material includes at least 75% nickel by weight and has a melting point of less than about 1100° C. The tungsten carbide pellets are substantially randomly dispersed throughout the matrix material. Furthermore, each sintered tungsten pellet includes a plurality of tungsten carbide particles bonded together with a binder alloy having a melting point greater than about 1200° C.

The features, advantages, and alternative aspects of the present invention will be apparent to those skilled in the art from a consideration of the following detailed description considered in combination with the accompanying drawings.

#### BRIEF DESCRIPTION OF THE DRAWINGS

While the specification concludes with claims particularly pointing out and distinctly claiming that which is regarded as the present invention, the advantages of this invention may be more readily ascertained from the following description of the invention when read in conjunction with the accompanying drawings in which:

FIG. 1 is a perspective view of a rotary type drill bit that includes cutting elements;

FIG. 2 is an enlarged view of a cutting element of the drill bit shown in FIG. 1;

FIG. 3 is a representation of a photomicrograph of an abrasive wear-resistant material that includes tungsten carbide particles substantially randomly dispersed throughout a matrix material;

FIG. 4 is an enlarged view of a tungsten carbide particle shown in FIG. 3;

FIG. 5 is a representation of a photomicrograph of an abrasive wear-resistant material that embodies teachings of the present invention and that includes tungsten carbide particles substantially randomly dispersed throughout a matrix;

FIG. 6 is an enlarged view of a tungsten carbide particle shown in FIG. 5;

FIG. 7A is an enlarged view of a cutting element of a drill bit that embodies teachings of the present invention;

FIG. 7B is a lateral cross-sectional view of the cutting element shown in FIG. 7A taken along section line 7B-7B therein;

FIG. 7C is a longitudinal cross-sectional view of the cutting element shown in FIG. 7A taken along section line 7C-7C therein;

FIG. 8A is a lateral cross-sectional view like that of FIG. 7B illustrating another cutting element of a drill bit that embodies teachings of the present invention;

FIG. 8B is a longitudinal cross-sectional view of the cutting element shown in FIG. 8A; and

FIG. 9 is a photomicrograph of an abrasive wear-resistant material that embodies teachings of the present invention and that includes tungsten carbide particles substantially randomly dispersed throughout a matrix.

#### DETAILED DESCRIPTION

The illustrations presented herein, with the exception of FIG. 9, are not meant to be actual views of any particular material, apparatus, system, or method, but are merely idealized representations which are employed to describe the present invention. Additionally, elements common between figures may retain the same numerical designation.

FIG. 5 represents a polished and etched surface of an abrasive wear-resistant material 54 that embodies teachings of the present invention. FIG. 9 is an actual photomicrograph of a polished and etched surface of an abrasive wear-resistant material that embodies teachings of the present invention. Referring to FIG. 5, the abrasive wear-resistant material 54 includes a plurality of sintered tungsten carbide pellets 56 and a plurality of cast tungsten carbide pellets 58 substantially randomly dispersed throughout a matrix material 60. Each sintered tungsten carbide pellet 56 and each cast tungsten carbide pellet 58 may have a generally spherical pellet configuration. The term "pellet" as used herein means any particle having a generally spherical shape. Pellets are not true spheres, but lack the corners, sharp edges, and angular projections commonly found in crushed and other non-spherical tungsten carbide particles.

Corners, sharp edges, and angular projections may produce residual stresses, which may cause tungsten carbide material in the regions of the particles proximate the residual stresses to melt at lower temperatures during application of the abrasive wear-resistant material 54 to a surface of a drill bit. Melting or partial melting of the tungsten carbide material during application may facilitate atomic diffusion between the tungsten carbide particles and the surrounding matrix material. As previously discussed herein, atomic diffusion between the matrix material 60 and the sintered tungsten carbide pellets 56 and cast tungsten carbide pellets 58 may embrittle the matrix material 60 in regions surrounding the tungsten carbide pellets 56, 58 and reduce the hardness of the tungsten carbide pellets 56, 58 in the outer regions thereof. Such atomic diffusion may degrade the overall physical properties of the abrasive wear-resistant material 54. The use of sintered tungsten carbide pellets 56 and cast tungsten carbide pellets 58 instead of conventional tungsten carbide particles that include corners, sharp edges, and angular projections may reduce such atomic diffusion, thereby preserving the physical properties of the matrix material 60, the sintered tungsten carbide pellets 56, and the cast tungsten carbide pellets 58 during application of the abrasive wear-resistant material 54 to the surfaces of drill bits and other tools.

The matrix material 60 may comprise between about 30% and about 50% by weight of the abrasive wear-resistant material 54. More particularly, the matrix material 60 may comprise between about 30% and about 35% by weight of the abrasive wear-resistant material 54. The plurality of sintered tungsten carbide pellets 56 may comprise between about 30% and about 55% by weight of the abrasive wear-resistant material 54. Furthermore, the plurality of cast tungsten carbide pellets 58 may comprise between about 15% and about 35% by weight of the abrasive wear-resistant material 54. For example, the matrix material 60 may be about 30% by weight of the abrasive wear-resistant material 54, the plurality of sintered tungsten carbide pellets 56 may be about 50% by weight of the abrasive wear-resistant material 54, and the plurality of cast tungsten carbide pellets 58 may be about 20% by weight of the abrasive wear-resistant material 54.

The sintered tungsten carbide pellets 56 may be larger in size than the cast tungsten carbide pellets 58. Furthermore, the number of cast tungsten carbide pellets 56 per unit volume of the abrasive wear-resistant material 54 may be higher than the number of sintered tungsten carbide pellets 58 per unit volume of the abrasive wear-resistant material 54.

The sintered tungsten carbide pellets 56 may include -20 ASTM mesh pellets. As used herein, the phrase "-20 ASTM

mesh pellets" means pellets that are capable of passing through an ASTM 20 mesh screen. Such sintered tungsten carbide pellets may have an average diameter of less than about 850 microns. The average diameter of the sintered tungsten carbide pellets 56 may be between about 1.1 times and about 5 times greater than the average diameter of the cast tungsten carbide pellets 58. The cast tungsten carbide pellets 58 may include -100 ASTM mesh pellets. As used herein, the phrase "-100 ASTM mesh pellets" means pellets that are capable of passing through an ASTM 100 mesh screen. Such cast tungsten carbide pellets may have an average diameter of less than about 150 microns.

As an example, the sintered tungsten carbide pellets 56 may include -60/+80 ASTM mesh pellets, and the cast tungsten carbide pellets 58 may include -100/+270 ASTM mesh pellets. As used herein, the phrase "-60/+80 ASTM mesh pellets" means pellets that are capable of passing through an ASTM 60 mesh screen, but incapable of passing through an ASTM 80 mesh screen. Such sintered tungsten carbide pellets may have an average diameter of less than about 250 microns and greater than about 180 microns. Furthermore, the phrase "-100/+270 ASTM mesh pellets," as used herein, means pellets capable of passing through an ASTM 100 mesh screen, but incapable of passing through an ASTM 270 mesh screen. Such cast tungsten carbide pellets 58 may have an average diameter in a range from approximately 50 microns to about 150 microns.

As another example, the plurality of sintered tungsten carbide pellets 56 may include a plurality of -60/+80 ASTM mesh sintered tungsten carbide pellets and a plurality of -120/+270 ASTM mesh sintered tungsten carbide pellets. The plurality of -60/+80 ASTM mesh sintered tungsten carbide pellets may comprise between about 30% and about 50% by weight of the abrasive wear-resistant material 54, and the plurality of -120/+270 ASTM mesh sintered tungsten carbide pellets may comprise between about 15% and about 20% by weight of the abrasive wear-resistant material 54. As used herein, the phrase "-120/+270 ASTM mesh pellets," as used herein, means pellets capable of passing through an ASTM 120 mesh screen, but incapable of passing through an ASTM 270 mesh screen. Such cast tungsten carbide pellets 58 may have an average diameter in a range from approximately 50 microns to about 125 microns.

Cast and sintered pellets of carbides other than tungsten carbide also may be used to provide abrasive wear-resistant materials that embody teachings of the present invention. Such other carbides include, but are not limited to, chromium carbide, molybdenum carbide, niobium carbide, tantalum carbide, titanium carbide, and vanadium carbide.

The matrix material 60 may comprise a metal alloy material having a melting point that is less than about 1100° C. Furthermore, each sintered tungsten carbide pellet 56 of the plurality of sintered tungsten carbide pellets 56 may comprise a plurality of tungsten carbide particles bonded together with a binder alloy having a melting point that is greater than about 1200° C. For example, the binder alloy may comprise a cobalt-based metal alloy material or a nickel-based alloy material having a melting point that is greater than about 1200° C. In this configuration, the matrix material 60 may be substantially melted during application of the abrasive wear-resistant material 54 to a surface of a drilling tool such as a drill bit without substantially melting the cast tungsten carbide pellets 58, or the binder alloy or the tungsten carbide particles of the sintered tungsten carbide pellets 56. This enables the abrasive wear-resistant material 54 to be applied to a surface of a drilling tool at lower temperatures to minimize atomic diffusion between the

sintered tungsten carbide pellets **56** and the matrix material **60** and between the cast tungsten carbide pellets **58** and the matrix material **60**.

As previously discussed herein, minimizing atomic diffusion between the matrix material **60** and the sintered tungsten carbide pellets **56** and cast tungsten carbide pellets **58**, helps to preserve the chemical composition and the physical properties of the matrix material **60**, the sintered tungsten carbide pellets **56**, and the cast tungsten carbide pellets **58** during application of the abrasive wear-resistant material **54** to the surfaces of drill bits and other tools.

The matrix material **60** also may include relatively small amounts of other elements, such as carbon, chromium, silicon, boron, iron, and nickel. Furthermore, the matrix material **60** also may include a flux material such as silicomanganese, an alloying element such as niobium, and a binder such as a polymer material.

FIG. 6 is an enlarged view of a sintered tungsten carbide pellet **56** shown in FIG. 5. The hardness of the sintered tungsten carbide pellet **56** may be substantially consistent throughout the pellet. For example, the sintered tungsten carbide pellet **56** may include a peripheral or outer region **57** of the sintered tungsten carbide pellet **56**. The outer region **57** may roughly include the region of the sintered tungsten carbide pellet **56** outside the phantom line **64**. The sintered tungsten carbide pellet **56** may exhibit a first average hardness in the central region of the pellet enclosed by the phantom line **64**, and a second average hardness at locations within the peripheral region **57** of the pellet outside the phantom line **64**. The second average hardness of the sintered tungsten carbide pellet **56** may be greater than about 99% of the first average hardness of the sintered tungsten carbide pellet **56**. As an example, the first average hardness may be about 91 on the Rockwell A scale and the second average hardness may be about 90 on the Rockwell A scale. Moreover, the fracture toughness of the matrix material **60** within the region **61** proximate the sintered tungsten carbide pellet **56** and enclosed by the phantom line **66** may be substantially similar to the fracture toughness of the matrix material **60** outside the phantom line **66**.

Commercially available metal alloy materials that may be used as the matrix material **60** in the abrasive wear-resistant material **54** are sold by Broco, Inc., of Rancho Cucamonga, Calif. under the trade names VERSALLOY® 40 and VERSALLOY® 50. Commercially available sintered tungsten carbide pellets **56** and cast tungsten carbide pellet **58** that may be used in the abrasive wear-resistant material **54** are sold by Sulzer Metco WOKA GmbH, of Barchfeld, Germany.

The sintered tungsten carbide pellets **56** may have relatively high fracture toughness relative to the cast tungsten carbide pellets **58**, while the cast tungsten carbide pellets **58** may have relatively high hardness relative to the sintered tungsten carbide pellets **56**. By using matrix materials **60** as described herein, the fracture toughness of the sintered tungsten carbide pellets **56** and the hardness of the cast tungsten carbide pellets **58** may be preserved in the abrasive wear-resistant material **54** during application of the abrasive wear-resistant material **54** to a drill bit or other drilling tool, thereby providing an abrasive wear-resistant material **54** that is improved relative to abrasive wear-resistant materials known in the art.

Abrasive wear-resistant materials that embody teachings of the present invention, such as the abrasive wear-resistant material **54** illustrated in FIGS. 5-6, may be applied to selected areas on surfaces of rotary drill bits (such as the rotary drill bit **10** shown in FIG. 1), rolling cutter drill bits

(commonly referred to as "roller cone" drill bits), and other drilling tools that are subjected to wear such as ream-while-drilling tools and expandable reamer blades, all such apparatuses and others being encompassed, as previously indicated, within the term "drill bit."

Certain locations on a surface of a drill bit may require relatively higher hardness, while other locations on the surface of the drill bit may require relatively higher fracture toughness. The relative weight percentages of the matrix material **60**, the plurality of sintered tungsten carbide pellets **56**, and the plurality of cast tungsten carbide pellets **58** may be selectively varied to provide an abrasive wear-resistant material **54** that exhibits physical properties tailored to a particular tool or to a particular area on a surface of a tool. For example, the surfaces of cutting teeth on a rolling cutter type drill bit may be subjected to relatively high impact forces in addition to frictional-type abrasive or grinding forces. Therefore, abrasive wear-resistant material **54** applied to the surfaces of the cutting teeth may include a higher weight percentage of sintered tungsten carbide pellets **56** in order to increase the fracture toughness of the abrasive wear-resistant material **54**. In contrast, the gage surfaces of a drill bit may be subjected to relatively little impact force but relatively high frictional-type abrasive or grinding forces. Therefore, abrasive wear-resistant material **54** applied to the gage surfaces of a drill bit may include a higher weight percentage of cast tungsten carbide pellets **58** in order to increase the hardness of the abrasive wear-resistant material **54**.

In addition to being applied to selected areas on surfaces of drill bits and drilling tools that are subjected to wear, the abrasive wear-resistant materials that embody teachings of the present invention may be used to protect structural features or materials of drill bits and drilling tools that are relatively more prone to wear.

A portion of a representative rotary drill bit **50** that embodies teachings of the present invention is shown in FIG. 7A. The rotary drill bit **50** is structurally similar to the rotary drill bit **10** shown in FIG. 1, and includes a plurality of cutting elements **22** positioned and secured within pockets provided on the outer surface of a bit body **12**. As illustrated in FIG. 7A, each cutting element **22** may be secured to the bit body **12** of the drill bit **50** along an interface therebetween. A bonding material **24** such as, for example, an adhesive or brazing alloy may be provided at the interface and used to secure and attach each cutting element **22** to the bit body **12**. The bonding material **24** may be less resistant to wear than the materials of the bit body **12** and the cutting elements **22**. Each cutting element **22** may include a polycrystalline diamond compact table **28** attached and secured to a cutting element body or substrate **23** along an interface.

The rotary drill bit **50** further includes an abrasive wear-resistant material **54** disposed on a surface of the drill bit **50**. Moreover, regions of the abrasive wear-resistant material **54** may be configured to protect exposed surfaces of the bonding material **24**.

FIG. 7B is a lateral cross-sectional view of the cutting element **22** shown in FIG. 7A taken along section line 7B-7B therein. As illustrated in FIG. 7B, continuous portions of the abrasive wear-resistant material **54** may be bonded both to a region of the outer surface of the bit body **12** and a lateral surface of the cutting element **22** and each continuous portion may extend over at least a portion of the interface between the bit body **12** and the lateral sides of the cutting element **22**.

## 11

FIG. 7C is a longitudinal cross-sectional view of the cutting element 22 shown in FIG. 7A taken along section line 7C-7C therein. As illustrated in FIG. 7C, another continuous portion of the abrasive wear-resistant material 54 may be bonded both to a region of the outer surface of the bit body 12 and a lateral surface of the cutting element 22 and may extend over at least a portion of the interface between the bit body 12 and the longitudinal end surface of the cutting element 22 opposite the polycrystalline diamond compact table 28. Yet another continuous portion of the abrasive wear-resistant material 54 may be bonded both to a region of the outer surface of the bit body 12 and a portion of the exposed surface of the polycrystalline diamond compact table 28 and may extend over at least a portion of the interface between the bit body 12 and the face of the polycrystalline diamond compact table 28.

In this configuration, the continuous portions of the abrasive wear-resistant material 54 may cover and protect at least a portion of the bonding material 24 disposed between the cutting element 22 and the bit body 12 from wear during drilling operations. By protecting the bonding material 24 from wear during drilling operations, the abrasive wear-resistant material 54 helps to prevent separation of the cutting element 22 from the bit body 12 during drilling operations, damage to the bit body 12, and catastrophic failure of the rotary drill bit 50.

The continuous portions of the abrasive wear-resistant material 54 that cover and protect exposed surfaces of the bonding material 24 may be configured as a bead or beads of abrasive wear-resistant material 54 provided along and over the edges of the interfacing surfaces of the bit body 12 and the cutting element 22.

A lateral cross-sectional view of a cutting element 22 of another representative rotary drill bit 50' that embodies teachings of the present invention is shown in FIGS. 8A and 8B. The rotary drill bit 50' is structurally similar to the rotary drill bit 10 shown in FIG. 1, and includes a plurality of cutting elements 22 positioned and secured within pockets provided on the outer surface of a bit body 12'. The cutting elements 22 of the rotary drill bit 50' also include continuous portions of the abrasive wear-resistant material 54 that cover and protect exposed surfaces of a bonding material 24 along the edges of the interfacing surfaces of the bit body 12' and the cutting element 22, as discussed previously herein in relation to the rotary drill bit 50 shown in FIGS. 7A-7C.

As illustrated in FIG. 8A, however, recesses 70 are provided in the outer surface of the bit body 12' adjacent the pockets within which the cutting elements 22 are secured. In this configuration, a bead or beads of abrasive wear-resistant material 54 may be provided within the recesses 70 along the edges of the interfacing surfaces of the bit body 12 and the cutting element 22. By providing the bead or beads of abrasive wear-resistant material 54 within the recesses 70, the extent to which the bead or beads of abrasive wear-resistant material 54 protrude from the surface of the rotary drill bit 50' may be minimized. As a result, abrasive and erosive materials and flows to which the bead or beads of abrasive wear-resistant material 54 are subjected during drilling operations may be reduced.

The abrasive wear-resistant material 54 may be used to cover and protect interfaces between any two structures or features of a drill bit or other drilling tool. For example, the interface between a bit body and a periphery of wear knots or any type of insert in the bit body. In addition, the abrasive wear-resistant material 54 is not limited to use at interfaces

## 12

between structures or features and may be used at any location on any surface of a drill bit or drilling tool that is subjected to wear.

Abrasives wear-resistant materials that embody teachings of the present invention, such as the abrasive wear-resistant material 54, may be applied to the selected surfaces of a drill bit or drilling tool using variations of techniques known in the art. For example, a pre-application abrasive wear-resistant material that embodies teachings of the present invention may be provided in the form of a welding rod. The welding rod may comprise a solid cast or extruded rod consisting of the abrasive wear-resistant material 54. Alternatively, the welding rod may comprise a hollow cylindrical tube formed from the matrix material 60 and filled with a plurality of sintered tungsten carbide pellets 56 and a plurality of cast tungsten carbide pellets 58. An oxyacetylene torch or any other type of welding torch may be used to heat at least a portion of the welding rod to a temperature above the melting point of the matrix material 60 and less than about 1200° C. to melt the matrix material 60. This may minimize the extent of atomic diffusion occurring between the matrix material 60 and the sintered tungsten carbide pellets 56 and cast tungsten carbide pellets 58.

The rate of atomic diffusion occurring between the matrix material 60 and the sintered tungsten carbide pellets 56 and cast tungsten carbide pellets 58 is at least partially a function of the temperature at which atomic diffusion occurs. The extent of atomic diffusion, therefore, is at least partially a function of both the temperature at which atomic diffusion occurs and the time for which atomic diffusion is allowed to occur. Therefore, the extent of atomic diffusion occurring between the matrix material 60 and the sintered tungsten carbide pellets 56 and cast tungsten carbide pellets 58 may be controlled by controlling the distance between the torch and the welding rod (or pre-application abrasive wear-resistant material), and the time for which the welding rod is subjected to heat produced by the torch.

Oxyacetylene and atomic hydrogen torches may be capable of heating materials to temperatures in excess of 1200° C. It may be beneficial to slightly melt the surface of the drill bit or drilling tool to which the abrasive wear-resistant material 54 is to be applied just prior to applying the abrasive wear-resistant material 54 to the surface. For example, an oxyacetylene and atomic hydrogen torch may be brought in close proximity to a surface of a drill bit or drilling tool and used to heat to the surface to a sufficiently high temperature to slightly melt or "sweat" the surface. The welding rod comprising pre-application wear-resistant material then may be brought in close proximity to the surface and the distance between the torch and the welding rod may be adjusted to heat at least a portion of the welding rod to a temperature above the melting point of the matrix material 60 and less than about 1200° C. to melt the matrix material 60. The molten matrix material 60, at least some of the sintered tungsten carbide pellets 56, and at least some of the cast tungsten carbide pellets 58 may be applied to the surface of the drill bit, and the molten matrix material 60 may be solidified by controlled cooling. The rate of cooling may be controlled to control the microstructure and physical properties of the abrasive wear-resistant material 54.

Alternatively, the abrasive wear-resistant material 54 may be applied to a surface of a drill bit or drilling tool using an arc welding technique, such as a plasma transferred arc welding technique. For example, the matrix material 60 may be provided in the form of a powder (small particles of matrix material 60). A plurality of sintered tungsten carbide pellets 56 and a plurality of cast tungsten carbide pellets 58

## 13

may be mixed with the powdered matrix material 60 to provide a pre-application wear-resistant material in the form of a powder mixture. A plasma transferred arc welding machine then may be used to heat at least a portion of the pre-application wear-resistant material to a temperature above the melting point of the matrix material 60 and less than about 1200° C. to melt the matrix material 60.

Plasma transferred arc welding machines typically include a non-consumable electrode that may be brought in close proximity to the substrate (drill bit or other drilling tool) to which material is to be applied. A plasma-forming gas is provided between the substrate and the non-consumable electrode, typically in the form a column of flowing gas. An arc is generated between the electrode and the substrate to generate a plasma in the plasma-forming gas. The powdered pre-application wear-resistant material may be directed through the plasma and onto a surface of the substrate using an inert carrier gas. As the powdered pre-application wear-resistant material passes through the plasma it is heated to a temperature at which at least some of the wear-resistant material will melt. Once the at least partially molten wear-resistant material has been deposited on the surface of the substrate, the wear-resistant material is allowed to solidify. Such plasma transferred arc welding machines are known in the art and commercially available.

The temperature to which the pre-application wear-resistant material is heated as the material passes through the plasma may be at least partially controlled by controlling the current passing between the electrode and the substrate. For example, the current may be pulsed at a selected pulse rate between a high current and a low current. The low current may be selected to be sufficiently high to melt at least the matrix material 60 in the pre-application wear-resistant material, and the high current may be sufficiently high to melt or sweat the surface of the substrate. Alternatively, the low current may be selected to be too low to melt any of the pre-application wear-resistant material, and the high current may be sufficiently high to heat at least a portion of the pre-application wear-resistant material to a temperature above the melting point of the matrix material 60 and less than about 1200° C. to melt the matrix material 60. This may minimize the extent of atomic diffusion occurring between the matrix material 60 and the sintered tungsten carbide pellets 56 and cast tungsten carbide pellets 58.

Other welding techniques, such as metal inert gas (MIG) arc welding techniques, tungsten inert gas (TIG) arc welding techniques, and flame spray welding techniques are known in the art and may be used to apply the abrasive wear-resistant material 54 to a surface of a drill bit or drilling tool.

While the present invention has been described herein with respect to certain preferred embodiments, those of ordinary skill in the art will recognize and appreciate that it is not so limited. Rather, many additions, deletions and modifications to the preferred embodiments may be made without departing from the scope of the invention as hereinafter claimed. In addition, features from one embodiment may be combined with features of another embodiment while still being encompassed within the scope of the invention as contemplated by the inventors. Further, the invention has utility in drill bits and core bits having different and various bit profiles as well as cutter types.

What is claimed is:

1. An abrasive wear-resistant material comprising the following materials in pre-application ratios:

a matrix material, the matrix material comprising between about 20% and about 50% by weight of the abrasive wear-resistant material, the matrix material comprising

## 14

at least 75% nickel by weight, the matrix material having a melting point of less than about 1100° C.; a plurality of -20 ASTM mesh sintered tungsten carbide pellets substantially randomly dispersed throughout the matrix material, the plurality of sintered tungsten carbide pellets comprising between about 30% and about 55% by weight of the abrasive wear-resistant material, each sintered tungsten carbide pellet comprising a plurality of tungsten carbide particles bonded together with a binder alloy, the binder alloy having a melting point greater than about 1200° C.; and

a plurality of -100 ASTM mesh cast tungsten carbide pellets substantially randomly dispersed throughout the matrix material, the plurality of cast tungsten carbide pellets comprising between about 15% and about 35% by weight of the abrasive wear-resistant material.

2. The abrasive wear-resistant material of claim 1, wherein the plurality of -20 ASTM mesh sintered tungsten carbide pellets comprises a plurality of -60/+80 ASTM mesh sintered tungsten carbide pellets, and wherein the plurality of -100 ASTM mesh cast tungsten carbide pellets comprises a plurality of -100/+270 ASTM mesh cast tungsten carbide pellets.

3. The abrasive wear-resistant material of claim 1, wherein the plurality of -20 ASTM mesh sintered tungsten carbide pellets comprises a plurality of -60/+80 ASTM mesh sintered tungsten carbide pellets and a plurality of -120/+270 ASTM mesh sintered tungsten carbide pellets, the plurality of -60/+80 ASTM mesh sintered tungsten carbide pellets comprising between about 30% and about 35% by weight of the abrasive wear-resistant material, the plurality of -120/+270 ASTM mesh sintered tungsten carbide pellets comprising between about 15% and about 20% by weight of the abrasive wear-resistant material.

4. The abrasive wear-resistant material of claim 1, further comprising niobium, the niobium being less than about 1% by weight of the abrasive wear-resistant material.

5. The abrasive wear-resistant material of claim 1, wherein the chemical composition of each -20 ASTM mesh sintered tungsten carbide pellet is at least substantially homogeneous throughout the pellet.

6. The abrasive wear-resistant material of claim 1, wherein the chemical composition of each -100 ASTM mesh cast tungsten carbide pellet is at least substantially homogeneous throughout the pellet.

7. The abrasive wear-resistant material of claim 1, wherein the matrix material further comprises at least one of chromium, iron, boron, and silicon.

8. The abrasive wear-resistant material of claim 1, wherein each -20 ASTM mesh sintered tungsten carbide pellet has a first average hardness in a central region of the pellet and a second hardness in a peripheral region of the pellet, the second hardness being greater than about 99% of the first hardness.

9. The abrasive wear-resistant material of claim 8, wherein the first hardness and the second hardness are greater than about 89 on a Rockwell A hardness scale.

10. The abrasive wear-resistant material of claim 1, wherein the plurality of -20 ASTM mesh sintered tungsten carbide pellets comprises a plurality of -60/+80 ASTM mesh sintered tungsten carbide pellets.

11. The abrasive wear-resistant material of claim 1, wherein the plurality of -100 ASTM mesh cast tungsten carbide pellets comprises a plurality of -100/+270 ASTM mesh cast tungsten carbide pellets.

## 15

12. An abrasive wear-resistant material comprising:  
 a matrix material, the matrix material comprising between  
 about 20% and about 50% by weight of the abrasive  
 wear-resistant material, the matrix material comprising  
 at least 75% nickel by weight, the matrix material  
 having a melting point of less than about 1100° C.;  
 a plurality of -60/+80 ASTM mesh sintered tungsten  
 carbide pellets substantially randomly dispersed  
 throughout the matrix material, the plurality of sintered  
 tungsten carbide pellets comprising between about  
 30% and about 35% by weight of the abrasive wear-  
 resistant material, each sintered tungsten carbide pellet  
 comprising a plurality of tungsten carbide particles  
 bonded together with a binder alloy, the binder alloy  
 having a melting point greater than about 1200° C.; and  
 a plurality of -100/+270 ASTM mesh cast tungsten  
 carbide pellets substantially randomly dispersed  
 throughout the matrix material, the plurality of cast  
 tungsten carbide pellets comprising between about  
 15% and about 20% by weight of the abrasive wear-  
 resistant material.

13. A tool for drilling a subterranean formation, comprising:

a bit body; and  
 an abrasive wear-resistant material over at least a portion  
 of the bit body, the abrasive wear-resistant material  
 comprising the following materials in pre-application  
 ratios:  
 a matrix material, the matrix material comprising  
 between about 20% and about 50% by weight of the  
 abrasive wear-resistant material, the matrix material  
 comprising at least 75% nickel by weight, the matrix  
 material having a melting point of less than about  
 1100° C.;  
 a plurality of -20 ASTM mesh sintered tungsten  
 carbide pellets substantially randomly dispersed  
 throughout the matrix material, the plurality of sintered  
 tungsten carbide pellets comprising between  
 about 30% and about 55% by weight of the abrasive  
 wear-resistant material, each sintered tungsten car-

10  
 15  
 20  
 25  
 30  
 35

## 16

bide pellet comprising a plurality of tungsten carbide  
 particles bonded together with a binder alloy, the  
 binder alloy having a melting point greater than  
 about 1200° C.; and  
 a plurality of -100 ASTM mesh cast tungsten carbide  
 pellets substantially randomly dispersed throughout  
 the matrix material, the plurality of cast tungsten  
 carbide pellets comprising between about 15% and  
 about 35% by weight of the abrasive wear-resistant  
 material.

14. The tool of claim 13, further comprising at least one  
 cutting element secured to the bit body.

15. The tool of claim 14, wherein the abrasive wear-  
 resistant material is disposed over an interface between the  
 bit body and the at least one cutting element.

16. The tool of claim 15, wherein the bit body comprises  
 a bit body having an outer surface and a pocket therein, at  
 least a portion of the at least one cutting element being  
 disposed within the pocket, the interface extending along  
 adjacent surfaces of the bit body and the at least one cutting  
 element.

17. The tool of claim 14, wherein the at least one cutting  
 element comprises a cutting element body and a diamond  
 compact table secured to an end of the cutting element body.

18. The tool of claim 13, wherein the plurality of -20  
 ASTM mesh sintered tungsten carbide pellets comprises a  
 plurality of -60/+80 ASTM mesh sintered tungsten carbide  
 pellets, and wherein the plurality of -100 ASTM mesh cast  
 tungsten carbide pellets comprises a plurality of -100/+270  
 ASTM mesh cast tungsten carbide pellets.

19. The tool of claim 13, wherein each -20 ASTM mesh  
 sintered tungsten carbide pellet has a first average hardness  
 in a central region of the pellet and a second hardness in a  
 peripheral region of the pellet, the second hardness being  
 greater than about 99% of the first hardness.

20. The tool of claim 19, wherein the first hardness and  
 the second hardness are greater than about 89 on a Rockwell  
 A hardness scale.

\* \* \* \* \*